

## UNITED STATES PATENT OFFICE

2,042,679

## METHOD OF MIXING RESINS WITH OTHER MATERIAL

Louis W. Murray and Ralph L. Seabury, Anderson, Ind., assignors, by mesne assignments, to General Motors Corporation, Detroit, Mich., a corporation of Delaware

No Drawing. Application May 29, 1930,  
Serial No. 457,504

7 Claims. (Cl. 106—22)

The present invention relates to a method of mixing resins such as "Bakelite" and similar compounds with finely shredded, powdered or granular material, either conductors or non-conductors.

5 Non-conductors may include wood flour, asbestos powder, shredded asbestos and shredded rags. Conductors may include graphite, coke and metal powders such as used for example in the manufacture of brushes for electric machines.

10 It is the object of the invention to devise a method of mixing resins and such materials as above referred to, which will be effective to secure a more intimate and homogeneous mixture of these materials in which the various ingredients 15 which constitute such mixture are more uniformly distributed than has been heretofore possible.

The methods heretofore employed the mixing of resins with powdered or granular material, such for instance as the graphite or copper powder used in the manufacture of brushes, have been principally two. According to the first of these, the resin and other materials which are used in forming the article are pulverized and are mixed in powdered form, in any suitable mixing device, 25 while dry. In carrying out the second method, the resin is dissolved in a volatile solvent such as benzol or alcohol or a mixture of the two. In this dissolved state, it is mixed with the other materials comprising the desired mixture, these materials being in powdered form. The solution is then evaporated in any suitable way to eliminate the volatile solvent and the residue is then adapted to be molded or dried in any desired manner.

30 The first of the methods above referred to is not altogether satisfactory because it is exceedingly difficult to secure a homogeneous mixture of the various ingredients which goes to make up the whole. In some parts of the mass certain of the ingredients will be found in greater proportions than in other parts and if powdered metal is used in the mixture as in the formation of a brush, it will be found that it is unevenly distributed throughout the mass, and the conductivity 35 of the brushes will not be uniform because of the unequal distributed copper particles. Therefore, because the first described method of mixing the various materials together is not altogether effective, it is found that a non-uniform product will be the result, whether it be a brush or some other element made from the mixture of materials.

40 The second method described is somewhat more effective to secure a uniform and intimate mixture of the various ingredients, but because of the use 45 of the volatile solvent for the binder the danger

from fire is great and the process expensive because the solvent is not recovered. According to the present invention, a method is devised which is effective to secure a uniform mixture and eliminates the fire hazard, while it is also much less 5 expensive because it eliminates the loss incurred by evaporation of the volatile solvent.

According to this invention, the materials which are being mixed are wet with lime water or some other alkali such as sodium or potassium hydroxide during the mixing process. Specifically, finely powdered graphite and finely powdered resin, such as powdered "Bakelite", are placed in any suitable mixing machine and the lime water, or some other alkaline solution, such as sodium 15 hydrate, sodium silicate or sodium carbonate is added slowly as the materials are mixed, until the mass in the mixing machine becomes a thick 20 paste. The effect of the alkaline solution is to soften the particles of the resin on the surface 25 thereof sufficiently to cause them to form an intimate mixture with the graphite.

The quantities of the materials employed will vary to some extent with the alkali employed, but if lime water is used, a suitable mixture for forming brushes is obtained from the following quantities of the various materials used: eighty-eight 30 parts graphite, ten parts "Bakelite" and two parts lime, by weight.

It will be noted that the addition of lime water 35 is not sufficient to cause the resin particles to be taken up in the solution, but since the lime water tends to dissolve the particles, the exterior thereof is softened. This causes a very intimate adhesion to take place between the various resin particles and graphite particles in the mixture. Any of the various alkaline solutions, such as above referred to, may be used instead of lime water with satisfactory results.

40 After addition of the lime water, the mixture may be washed, filtered and dried in any suitable way. The dried mixture may then be used in the manufacture of brushes or for any other purpose desired.

45 Also, instead of employing lime water to soften the "Bakelite", the invention contemplates the use of calcium oxide and plain water to effect the same result. When calcium oxide is employed, the proportions which have been found to give good results in the formation of a brush for an electric machine are eighty-eight pounds graphite, ten pounds resin and two pounds of calcium oxide. It will be understood of course that if the materials are being mixed for use in the 50 55

formation of different articles, the proportions of the various materials may not be the same. In carrying out the method, the calcium oxide is added as a powder to the powdered graphite and resin during the mixing of the latter and all three are then mixed in the mixing machine while water is added slowly until a thick paste is formed of substantially the same consistency as the paste secured when employing lime water. The action 5 of the calcium oxide with water is substantially the same as when lime water is used, the water and oxide forming calcium hydroxide during the process of mixing the mass. Subsequent to this operation the mixture may be filtered, washed 10 and dried as above set forth. As has been pointed out, the advantages of this method of mixing resins and other materials are apparent. A better mixture is secured than with methods formerly used, the method is less expensive than that in which the resin is dissolved in a volatile solvent, and a better and more uniform product may, 15 therefore, be obtained at a lower cost than with former methods.

While the form of embodiment of the present 20 invention as herein disclosed, constitutes a preferred form, it is to be understood that other forms might be adopted, all coming within the scope of the claims which follow.

What is claimed is as follows:

80 1. The process of mixing resins with granular or powdered materials which consists in mixing dry powdered resin with some other dry powdered material, adding a quantity of alkaline solution during the mixing operation sufficient to 25 soften the surface of the particles of resin but insufficient to dissolve said particles, washing 30

sufficient to dissolve the resin, washing and filtering the paste and drying the washed residue.

3. The process of mixing resins with granular or powdered materials which includes the steps of mixing dry powdered resin with other dry powdered materials and adding a quantity of alkaline solution during the mixing operation sufficient to cause the resin to become sticky but insufficient to dissolve the resin. 5

4. The method of mixing materials for forming 10 brushes for electric machines which includes the steps of mixing substantially eighty-eight parts powdered graphite with substantially ten parts "Bakelite" powder, and adding two parts lime in the form of lime water during the mixing 15 operation.

5. The process of mixing resins with granular or powdered materials which consists in mixing 20 powdered resin, calcium oxide powder and other powdered or granular material, adding a quantity of water during the mixing operation sufficient to react with the calcium oxide and soften the resin but insufficient to dissolve the resin, washing and filtering the mixture and driving 25 the residue.

6. The method of mixing resins with granular or powdered materials which includes the steps of mixing powdered resin with other powdered materials, and adding a quantity of calcium oxide and water to such mixture during the mixing 30 operation sufficient to soften the resin but insufficient to dissolve the resin.

7. The method of mixing materials for forming 35 brushes for electric machines which includes the steps of mixing substantially eighty-eight parts powdered graphite, ten parts "Bakelite" powder, two parts calcium oxide powder and